

W. S. ROWLAND.  
ANNEALING APPARATUS AND PROCESS.  
APPLICATION FILED JUNE 26, 1917.

1,268,155.

Patented June 4, 1918.



INVENTOR.

BY

*H. E. Hart*  
H. E. Hart  
ATTORNEY.

# UNITED STATES PATENT OFFICE.

WILLIAM S. ROWLAND, OF NEW BRITAIN, CONNECTICUT, ASSIGNOR TO THE STANLEY WORKS, OF NEW BRITAIN, CONNECTICUT, A CORPORATION OF CONNECTICUT.

## ANNEALING APPARATUS AND PROCESS.

1,268,155.

Specification of Letters Patent. Patented June 4, 1918.

Application filed June 26, 1917. Serial No. 177,132.

*To all whom it may concern:*

Be it known that I, WILLIAM S. ROWLAND, a citizen of the United States, and a resident of New Britain, in the county of 5 Hartford, State of Connecticut, have invented certain new and useful Improvements in Annealing Apparatus and Processes, of which the following is a specification.

10 This invention relates generally to the annealing of metals in strip form, as distinguished from what is commonly called wire stock and of varying cross-sectional size and shape. The object of this invention 15 is to provide an improved apparatus and process for annealing by which a product of the desired characteristics may be produced continuously at a relatively fast rate of production. It relates to a type of apparatus where the strip is moved continuously 20 through the annealing apparatus.

In the drawings—

Figure 1 is a diagrammatic side elevation of an apparatus for carrying out the invention.

Fig. 2 is a cross-sectional view on the line 2—2 of Fig. 1.

Referring to the drawings:—A denotes the complete apparatus from end to end 30 which will be hereinafter referred to as a chamber comprising a tubular section B and a box-like section C, within which are located water-jacketed cooling drums D, D, E, denotes a furnace surrounding a portion 35 of the tubular section B and in which any heat-producing agent, as gas, may be burned. F, denotes the entrance end of the chamber and G denotes the exit end which will be seen to be arranged in the same plane 40 at the same level and, as here shown, below the heated part of the section B. K, K indicate gas inlets provided near to the entrance and exit of the chamber. S indicates the strip of metal which is being annealed. 45 It is understood that the metal is being continuously uncoiled and straightened and then passed through the chamber, annealed, cooled and then taken out and coiled up.

As seen in Fig. 2, the section B of the 50 chamber is tubular and the flat strip bears only at its edges, which term is meant to exclude any portion of the surface of the strip, thus avoiding any liability of scratching or marring the surface of the strip. All 55 parts of the chamber from entrance to exit

are in free and open communication and filled with a dry non-oxidizing gas envelop. An excess supply of gas is provided at both the entrance and exit of the chamber through the inlets, K K; this gas, or substantially all of it, flowing into the chamber near and then immediately out of the entrance and exit, effectually providing what is in substance a gas seal at both the entrance and exit to prevent the ingress of 60 air or other oxidizing agencies. A convenient way of disposing of the gas as it leaves the entrance and exit is to burn it.

The arrows at each end of the apparatus show the way in which the gas passes into 65 and immediately out of each end. Under normal conditions the best practice calls for the inflow of gas at K, K at equal rates of flow. By maintaining the entrance and exit at the same level any tendency of the gas 70 within the chamber to flow is overcome. The entrance and exit should be out of the plane of the heated part of the chamber and conveniently below, as here illustrated.

This apparatus is designed particularly 75 for use in annealing cold rolled steel, which is produced of accurate gage and with a highly polished surface. Where this cold rolled steel is to be annealed, it is desirable 80 that, after the annealing process, the surface shall be as bright and highly polished as 85 when it enters the annealing apparatus and by the apparatus and process herein above disclosed, a uniform product is produced having all of the desired characteristics to a 90 very marked degree.

Important features of the apparatus and process consist in maintaining the gas envelop in a substantially non-flowing or static 95 condition; constantly providing a supply of non-oxidizing gas at the entrance and exit and thus sealing these points to prevent the ingress of an oxidizing atmosphere; so supporting the strip as it travels through the chamber, and especially through the tubular 100 portion of the chamber, as to avoid subjecting its surface to any rubbing action which might mar it when it is hot, this being accomplished by so adjusting the shape of the chamber section B to the cross-sectional 105 shape of the strip as to have the strip supported at its edges. It is of course understood that that part of the tubular section B within the furnace is heated and the gas and metal within the tubular section is thus 110

heated. The water-jacketed drums D, D, about which the strip is wound, provide a proper cooling agency and reduce the temperature of the metal before its passage into the air to such a point that oxidization will not take place.

I claim as my invention:—

1. In an apparatus for annealing metals, a chamber provided with heating and cooling sections, the cross-sectional shape of said heating chamber being so related to the cross-sectional shape of the strip continuously passing therethrough so that said strip shall be supported within said chamber by the contact of its edges with the inner wall of said chamber.

2. That improvement in the art of annealing metals where a strip is continuously moved through an annealing chamber which consists in supporting said strip at its edges without any surface contact while moving through a portion of said chamber and thereby preventing the marring of any portion of the surface of said strip.

3. That step in the art of continuously annealing a strip of metal by passing it through a chamber comprising heating and cooling sections supplied with a suitable non-oxidizing atmosphere, which consists in introducing a non-oxidizing gas into said chamber near its entrance and exit, and permitting the greater part of said gas to escape through the said entrance and exit.

4. In an apparatus for annealing metals by passing a strip continuously through an annealing chamber, a chamber comprising heating and cooling sections with its entrance and exit arranged at substantially the

same level and out of the plane of the heating section, a substantially non-flowing non-oxidizing atmosphere within said chamber, and means at the entrance and exit for continuously supplying a non-oxidizing gas.

5. In an apparatus for annealing metals by passing a strip continuously through an annealing chamber, a chamber comprising heating and cooling sections with its entrance and exit arranged at substantially the same level and out of the plane of the heating section, a substantially non-flowing, non-oxidizing atmosphere within said chamber, and means at the entrance and exit for continuously supplying a non-oxidizing gas at substantially equal rates of flow.

6. In an apparatus for annealing metals by passing a strip continuously through an annealing chamber, an annealing chamber comprising heating and cooling sections in open communication with one another, a non-oxidizing atmosphere within said chamber, and an auxiliary supply of non-oxidizing gas at the entrance to and exit from said chamber to constitute a gas seal at said points.

7. In an apparatus for annealing metals by passing a strip continuously through an annealing chamber, an annealing chamber comprising heating and cooling sections in open communication with one another, a substantially non-flowing, non-oxidizing gas filling said chamber, and a gas seal at the entrance to and the exit from said chamber.

WILLIAM S. ROWLAND.

Witnesses:

ALMA STROMQUIST,  
W. E. DOANE.